

Patented Nov. 4, 1924.

1,513,793

## UNITED STATES PATENT OFFICE.

PERCY A. E. ARMSTRONG, OF LOUDONVILLE, AND RALPH P. DE VRIES, OF NEWTONVILLE, NEW YORK, ASSIGNEES, BY DIRECT AND MESNE ASSIGNMENTS, TO LUDLUM STEEL COMPANY, OF WATERVLIET, NEW YORK, A CORPORATION OF NEW JERSEY.

### TOUGH STABLE-SURFACE ALLOY STEEL.

No Drawing.

Application filed February 1, 1921. Serial No. 441,641.

To all whom it may concern:

Be it known that we, PERCY A. E. ARMSTRONG, a subject of the King of Great Britain, and a resident of Loudonville, county 5 of Albany, and State of New York, and RALPH P. DE VRIES, a citizen of the United States, and a resident of Newtonville, county of Albany, and State of New York, have invented a new and useful Tough 10 Stable-Surface Alloy Steel, of which the following is a specification.

The invention relates to alloy steel. The alloy steel of the present invention has high surface stability, that is to say, has high 15 resistance to agents tending to produce corroding, rusting, staining and the like, and also is markedly high in toughness and mechanical strength as indicated by ductility and impact tests, for example, making 20 it particularly valuable for wrought metal articles which are to have high mechanical strength as well as highly stable surface characteristics.

The improved alloy steel contains principally iron, carbon, chromium, silicon and nickel, with more or less traces of manganese, phosphorus, etc., which are present in substantially all steels. With stable surface alloy steel containing principally iron, 25 carbon, chromium and silicon as disclosed in Patent No. 1,322,511 of Nov. 25th, 1919, to said Armstrong, the addition of nickel is of relatively small importance so far as the stable surface characteristics of the alloy 30 steel are concerned, though as is stated therein, some nickel can be added without substantial detriment to the stable surface qualities.

Where high mechanical strength and 35 toughness are of importance as well as high surface stability, we substitute another metal of the iron group, preferably nickel, for part of the iron in the alloy of said Armstrong patent, thereby increasing the toughness 40 of the alloy. Any tendency toward loss of surface stability produced by the substitution of nickel for part of the iron, such as results to some extent, for example, in respect to degree of resistance to rusting and 45 to the action of strong nitric acid, is compensated where tough material is required

by the increased toughness obtained. When the proportion of silicon is increased along with the substitution of nickel for a part of the iron tougher material can be obtained 55 with practically no loss whatever of surface stability.

This can best be understood from the following example: An alloy steel containing carbon .5%, chromium 17%, silicon 2%, and the rest principally iron has better resistance to rusting than the same alloy with 15-25% of nickel and correspondingly less iron, but the toughness of the latter alloy is greater. 60 With increase of the silicon to about 5% and without the nickel, an alloy is obtained of extremely high surface stability, but its physical properties are not so good as with the lower silicon. If 15-25% of nickel is incorporated in this last material in the 65 place of a corresponding quantity of iron, giving an alloy containing carbon .5%, chromium 17%, silicon 5%, nickel 15-25%, and the remainder principally iron, the surface stability, while reduced as compared 70 with the same material without the nickel, is about as good as with the alloy first-named in this paragraph, and the material is tough, and while comparatively hard to machine can nevertheless be machined with 75 the use of the proper tools.

The carbon of the alloy steel should be from about .05% to about .50%. Where the carbon is high, nickel does not add substantially to the toughness of the alloy steel. 80

The silicon content of the alloy steel is from about .75% to about 6% and preferably from about 1.5% to about 4.5%. With less than .75% the stable surface effect of silicon is relatively inconsiderable and with silicon above about 6%, the desirable toughness is reduced.

The chromium may be from about 5% to about 25%.

The nickel may be from about 4% to 95 about 30%, replacing a corresponding amount of iron.

Some examples of good alloy steel within the scope of our invention are given in the following table which is intended to serve 100 only as affording an understanding of some of the alloy steels within the scope of the

invention and not for limitation of the invention:

| 5  | Carbon.      | Chro-<br>mium. | Silicon.     | Nickel.      | Iron.                        |
|----|--------------|----------------|--------------|--------------|------------------------------|
|    | Per<br>cent. | Per<br>cent.   | Per<br>cent. | Per<br>cent. |                              |
| 10 | .40          | 17             | 3            | 15           | Principal part of remainder. |
|    | .35          | 16             | 4.5          | 16           | Principal part of remainder. |
|    | .50          | 16             | 5            | 20           | Principal part of remainder. |
|    | .55          | 12             | 4            | 25           | Principal part of remainder. |
|    | .30          | 20             | 3.5          | 30           | Principal part of remainder. |
|    | .30          | 8              | 2            | 10           | Principal part of remainder. |
|    | .40          | 5              | 3            | 15           | Principal part of remainder. |

The alloy steel of the present invention, particularly with over about 8% of nickel, appears to be generally austenitic in character. Sharp cutting tools should be used in machining it, and any rubbing action such as takes place in sawing for example, is preferably to be avoided. It should be noted that the inclusion of nickel in the alloy steel makes it more non-magnetic, and that in general in order to obtain equivalent stable surface characteristics with the inclusion of nickel, the proportion of silicon should be correspondingly increased as pointed out above, the resistance to attack by corrosive agents being increased by the addition of silicon that is made possible by the use of nickel, and this without undue loss or toughness. Where the silicon content is increased along with increase in the nickel content, the material, while austenitic in character as above stated, is of such character of austenite that it can be more readily machined than is the case where the same nickel and chromium are used with lower silicon. Where the alloy steel without the nickel does not tarnish upon exposure to weak acids such as vinegar, fruit juices and the like, and particularly where it contains over 13% of chromium and silicon taken together, the replacement of a portion of the iron by nickel as described herein to produce increased toughness may be carried out without causing the material to tarnish under such conditions.

The alloy steel of the present invention is adapted for a large number of uses requiring surface stability and toughness. Among numerous other uses, the following may be briefly referred to, but without limitation thereto: turbine bucket blades, ball bearings, balls, glass molds, shafts for machinery, cutlery, acid resisting material, non-

magnetic steels, automobile valves, rifle barrels, heat resisting material and electrical resistance elements. The specific resistance of the alloy steel of the present invention is about the same as that of the alloy steel of the Armstrong patent above referred to. The substitution of nickel for part of the iron does not appear to produce material change in conductivity when the alloy steel is made use of for electrical resistance or heating elements.

We claim:

1. A tough alloy steel of high surface stability containing carbon about .05% to about .50%, chromium from about 5% to about 25%, silicon from about 1.5% to about 6%, nickel from about 4% to about 30%, and the principal portion of the remainder iron. 70

2. A tough alloy steel having high surface stability, containing carbon about .05% to about .50%, chromium from about 8% to about 20%, silicon from about 1.5% to about 4.5%, nickel from about 4% to about 30%, and the principal portion of the remainder iron. 75

3. A tough alloy steel of high surface stability, comprising carbon from about .05% to about .5%, chromium from about 15% to about 20%, silicon from about 1.5% to about 4.5%, nickel from about 15% to about 30%, and the principal portion of the remainder iron. 85

4. Tough stable surface alloy steel comprising carbon about .05% to about .50%, chromium about 17%, silicon from about 1.5% to about 5%, nickel about 15% and the principal portion of the remainder iron. 90

5. Wrought metal articles having high surface stability and toughness, and made from alloy steel in accordance with claim 1. 95

6. Wrought metal articles having high surface stability and toughness, and made from alloy steel in accordance with claim 2. 100

7. Wrought metal articles having high surface stability and toughness, and made from alloy steel in accordance with claim 3.

8. Wrought metal articles having high surface stability and toughness, and made from alloy steel in accordance with claim 4. 105

In testimony that we claim the foregoing, we have signed our names hereto.

PERCY A. E. ARMSTRONG.  
RALPH P. DE VRIES.